

May 19, 1959

L. M. NIJLAND ET AL

2,887,629

TRANSISTOR

Filed Feb. 13, 1957



INVENTORS  
LOUIS MARIUS NIJLAND  
JAN ADRIANUS MANINTVELD

BY *Frank R. Jefco*  
AGENT

## 1

2,887,629

## TRANSISTOR

Louis Marius Nijland and Jan Adrianus Manintveld, Eindhoven, Netherlands, assignors, by mesne assignments, to North American Philips Company, Inc., New York, N.Y., a corporation of Delaware

Application February 13, 1957, Serial No. 639,951

Claims priority, application Netherlands  
February 29, 1956

8 Claims. (Cl. 317—234)

The invention relates to a method of producing a semi-conductive electrode system, more particularly a transistor, in which a semi-conductive body for example of germanium or silicon is provided with at least one rectifying electrode and one ohmic connection, this structure being then etched and housed in an envelope. The invention furthermore relates to a semi-conductive electrode system or device, more particularly a transistor housed in a vacuum-tight envelope.

The invention is found to be of particular use for transistors, for the purpose of increasing the current amplification factor  $\alpha_{cb}$ , which is defined by the equation:

$$\alpha_{cb} = \left( \frac{\delta I_c}{\delta I_b} \right) V_c$$

wherein  $I_c$  and  $I_b$  denote the collector current and the base current respectively, measured at a constant collector voltage  $V_c$ .

It is already known that the current amplification factor of germanium transistors and more particularly that of silicon transistors can be enhanced by coating the semi-conductive surface with a layer of oxidizing material, for example, of lead minium, zinc chromate or strontium chromate and that organic compounds may be used for this purpose. However, experiments have proved that transistors thus manufactured are often not stable, especially at high temperatures.

The invention has for its object to provide a method of producing a semi-conductive electrode system having a high current amplification factor and great stability. It has furthermore the advantage that the surface of the semi-conductive body can be provided in a simple manner with very thin layers, even layers of molecular thickness, producing these favourable effects.

In accordance with the invention the semi-conductive body with its electrode and ohmic connection is, after the etching operation, introduced into a space containing at least one of the halogens and/or their hydrates with the exception of elemental fluorine. The element fluorine is excepted, since it is unserviceable owing to its great reactivity. In practice it has been found that almost immediately an increase in the current amplification factor is obtained, if the space into which the semi-conductive body is introduced contains even a very small quantity of vapour of one or more of these elements and compounds. The effect aimed at by the invention is therefore also realized if the milieu or atmosphere contains a dissociating substance capable of producing a marked vapour pressure of the halogens and/or the hydro-halides. It should further be noted, that the results obtainable by the method according to the invention are in general not dependent upon the special etching solution employed.

Particularly suitable are found to be hydrochloric acid and hydro-fluoric acid. The effect is further increased if the space contains, in addition, water vapour.

A particular embodiment of the invention consists in that the semi-conductive body with its electrode and ohmic connection is accommodated in a vacuum-tight

## 2

envelope containing at least one of the halogens and of their hydrates, with the exception of the element fluorine. The envelope may, moreover, contain water vapour. According to a further aspect of the invention an additional effect is obtained, if, before the envelope is definitely sealed, the gaseous mixture contained therein is pumped off, preferably to a pressure of less than  $10^{-2}$  mm. Hg.

Although the invention is not restricted to its use with a special semi-conductive substance, it is of particular importance with semi-conductive electrode systems, for example alloy transistors, of which the semi-conductive body is made of silicon, since the conventional means, which yielded satisfactory values of the current amplification factor with germanium, do not give satisfactory results with silicon.

In one embodiment of a semi-conductive electrode system, more particularly a transistor according to the invention, the vacuum-tight envelope contains at least one of the halogens and/or one of their compounds with hydrogen, with the exception of the element fluorine. The envelope may furthermore contain water vapour.

It should be noted, that this gaseous atmosphere affects favourably not only transistors, but will yield similar results with other semi-conductive electrode systems, when the method according to the invention is employed.

One embodiment of a semi-conductive electrode system according to the invention, to which the invention is however not limited, will now be described with reference to the sole figure of the accompanying drawing, which shows, in cross-section, a transistor according to the invention.

Referring now to the figure, a transistor comprises a thin semi-conductive disc 1, provided with an emitter electrode 2, a collector electrode 3 and an ohmic annular base connection 4. The electrodes 2, 3 and the ohmic connection 4 are each connected to supply conductors 5, 6, 7 passing through a glass pinch 8, and are passed to the outside through the glass base 9, to which a glass bulb 10 is sealed. The envelope (9, 10) contains for instance dry HCl vapour at a pressure of about  $10^{-4}$  mm. Hg.

The method according to the invention will now be described more fully with reference to a few examples.

## Example 1

An alloy transistor comprising a semi-conductive body consisting of p-type silicon, provided with a base connection, consisting of an alloy of 90% by weight of indium and 10% by weight of copper, and further provided with an emitter electrode and a collector electrode, both consisting of 75% by weight of gold and 25% by weight of antimony, was etched in a bath containing a mixture of a 52% aqueous solution of hydrofluoric acid and a 97% aqueous solution of nitric acid in the volume ratio 1:3, and subsequently washed in streaming, distilled deionized water and dried. After measurement of the current amplification factor  $\alpha_{cb}$ , which turned out to be 4.5, the transistor was arranged in a glass envelope containing dry HCl. Owing to this treatment the current amplification factor  $\alpha_{cb}$  rose almost immediately to 27. During the subsequent pumping off  $\alpha_{cb}$  increased further and attained a maximum value of 31.5 at a pressure of about  $10^{-4}$  mm. Hg, after which the glass envelope was sealed tight. In order to check the stability of the transistor the assembly was then heated, whereby  $\alpha_{cb}$  increased continuously and reached a value of 37 at 180° C. During cooling to room temperature the same range was reversed, which confirms the stability of the transistor.

## Example 2

A silicon alloy transistor such as described in Example 1 was introduced after the etching operation into a space,

containing apart from HF also water vapour, of which the vapour pressure was about one hundredth of that of HF. Before this treatment the current amplification factor  $\alpha_{cb}$  was 6; after this treatment it had increased to 25. The transistor was then housed in a vacuum-tight envelope and heated to 180° C., at which temperature  $\alpha_{cb}$  was 35. After cooling to room temperature  $\alpha_{cb}$  was again 25, which confirms the stability of the transistor.

*Example 3*

Of an alloy transistor such as described in Example 1 the current amplification factor  $\alpha_{cb}$  was 5 after the etching operation. The transistor was then introduced into a space containing dry HCl; after this treatment  $\alpha_{cb}$  had increased to 27. By adding water vapour to an amount of about 1% relative to the HCl  $\alpha_{cb}$  rose to a value 30.

*Example 4*

An alloy transistor comprising a semi-conductive body consisting of n-type germanium, provided with a base electrode consisting of an alloy of 97% by weight of tin and 3% by weight of antimony, and further provided with an emitter electrode and a collector electrode, both consisting of indium, was etched in a bath composed of 2 volume parts 52% aqueous solution of HF, 2 volume parts 97% aqueous solution of HNO<sub>3</sub>, and 5 volume parts H<sub>2</sub>O, and subsequently washed in distilled water and dried. The current amplification factor amounted to 30 after this etching treatment. The transistor was then sealed in a glass envelope containing HF and water vapour. After this treatment  $\alpha_{cb}$  had increased to 90. During the subsequent heating  $\alpha_{cb}$  rose to a value 100 at a temperature of 70° C. During the cooling to room temperature the same range was reversed, which confirms the stability of the transistor.

*Example 5*

An alloy transistor such as described in Example 1, had a current amplification factor  $\alpha_{cb}$  of 2.7 after the etching operation. The transistor was then introduced into an envelope containing apart from bromine vapour, water vapour. Thus  $\alpha_{cb}$  increased to 18.5. During the subsequent heating  $\alpha_{cb}$  increased further to obtain a value 24 at 180° C. After cooling to room temperature  $\alpha_{cb}$  decreased practically to the initial value viz. 17.5.

What is claimed is:

1. A semi-conductive device comprising an etched semi-conductive body with plural electrode connections to said body and possessing a current amplification factor whose value depends on the surrounding atmosphere, a sealed envelope enclosing the body with its connections, and an atmosphere in said envelope comprising water vapor and

a substance selected from the group consisting of chlorine, bromine, iodine, and hydrogen compounds of the latter and of fluorine.

5 2. A semi-conductive device comprising an etched semi-conductive body selected from the group consisting of germanium and silicon and with ohmic and rectifying electrode connections to said body, a vacuum-tight sealed envelope enclosing the body with its connections, and an atmosphere in said envelope comprising water vapor and a substance selected from the group consisting of chlorine, bromine, iodine and hydrogen compounds of the latter and of fluorine.

10 3. A device as set forth in claim 2 wherein the atmosphere is at a pressure below 10<sup>-2</sup> mm. of mercury.

15 4. A device as set forth in claim 2 wherein the substance is hydrochloric acid.

20 5. A semi-conductive device comprising an etched semi-conductive body selected from the group consisting of germanium and silicon with ohmic and rectifying electrode connections to said body, a vacuum-tight sealed envelope enclosing the body with its connections, and an atmosphere in said envelope comprising a substance selected from the group consisting of hydrofluoric acid and hydrochloric acid.

25 6. A method manufacturing a semi-conductive device comprising a semi-conductive body and plural electrode connections to said body and possessing a current amplification factor whose value depends on the surrounding atmosphere, comprising etching the body, and thereafter

30 introducing the body with its electrode connections into an atmosphere containing water vapor and a substance selected from the group consisting of chlorine, bromine, iodine, and hydrogen compounds of the latter and of fluorine.

35 7. A method of manufacturing a semi-conductive device comprising a semi-conductive body selective from the group consisting of germanium and silicon and having ohmic and rectifying electrode connections to said body, comprising etching the body, and thereafter introducing the body with its electrode connections into an atmosphere containing water vapor and a substance selected from the group consisting of chlorine, bromine, iodine, and hydrogen compounds of the latter and of fluorine.

40 8. A method as set forth in claim 7 wherein the atmosphere is partly removed and then the body with its connections sealed-off in a vacuum-tight envelope.

**References Cited** in the file of this patent

**UNITED STATES PATENTS**

50 2,812,480 Ellis ----- Nov. 5, 1957